

Oct. 11, 1932.

H. WOODHEAD ET AL

1,882,352

PROCESS OF FORMING HOLLOW BRACING UNITS

Filed July 28, 1926

2 Sheets-Sheet 1



Inventors  
Clinton W. Stover  
Harry Woodhead  
By Bates, Macklin,  
Golick & Coare Attorneys

Oct. 11, 1932.

H. WOODHEAD ET AL

1,882,352

PROCESS OF FORMING HOLLOW BRACING UNITS

Filed July 28, 1926

2 Sheets-Sheet 2



FIG. 11



Inventors  
Clinton W. Stover,  
Harry Woodhead  
By Bates, Macklin,  
Golick & Tamm Attorneys

## UNITED STATES PATENT OFFICE

HARRY WOODHEAD AND CLINTON W. STOVER, OF CLEVELAND, OHIO

## PROCESS OF FORMING HOLLOW BRACING UNITS

Application filed July 28, 1926. Serial No. 125,396.

This invention relates to a process for making a combined tube and bracket, and is concerned particularly with taking a drawn steel tube of any desired length, and so working the metal on one or both ends that we may produce a compressed forged steel bracket or brackets integral with the tube, the bracket by reason of having the characteristics of forged steel being stronger than the tube itself.

The object of the invention is to provide a process for upsetting and flanging a tube, which process will require but a small number of operations and which will result in forming an unusually strong one piece bracket without waste as compared to forging brackets from slugs.

It is essential that we cause a longitudinal flow of the metal of the tube, first to provide thickness of metal and second to increase the strength of the metal by such upsetting or forging operations. Further refinements include the formation of depressions in the upset end of the tube during the first operation so that during the second operation the flanges are more easily formed and are stronger. The process includes the making of machine pads or slight bosses on the forged portion or portions, these being provided in our process by the use of corresponding cavities in the forming die members.

In carrying out our process we may support the tube simultaneously with the longitudinal compression on the end thereof just below the portion of the metal which is caused to flow, in order that, at the point of juncture between the tube and bracket, the tube itself may remain undistorted and will hold its position even though a very great longitudinal compression is applied in upsetting the end of the tube. Our process preferably includes two major steps, namely, first placing the heated tube in a female die having cavities of different diameters joined by tapering surfaces and forcing downwardly upon the end of the tube by a male die to cause the heated metal to flow and fill the cavity formed between the male and female dies; and second to support the thus upset tube in another female die and further com-

press the upset end, thereby causing the formation of flanges integral and joined to the tube by a thickened or webbed reinforce portion, also of forged metal.

In the drawings Fig. 1 is a cross sectional view through a cooperating set of dies with the end of a heated tube therein ready to be upset; Fig. 2 is a fragmentary side elevation of one form of male die; Fig. 3 is a cross sectional view similar to Fig. 1 showing the relative position of the dies at the end of the first operation; Figs. 4, 5 and 6 are fragmentary perspective views of upset tubes for forming flanges of different character; Fig. 7 is a sectional perspective view of the male finishing die; Fig. 8 shows the male and female finishing dies just beginning to form the flanges; Fig. 9 is a fragmentary cross sectional view through the same dies at the completion of the flange forming operation; Fig. 10 is a fragmentary perspective view of a female finishing die formed to provide bracing webs beneath the flanges; Fig. 11 is a fragmentary cross sectional view illustrating the formation of such bracing webs; Fig. 12 shows the finished forgings as produced by the dies shown in Fig. 8; Fig. 13 is a similar view showing different flanges and webs; Fig. 14 is a sectional perspective view through the end of a flanged tube showing machine pads; Fig. 15 shows a completely formed bracket such as might be formed by the blank shown in Fig. 6; Fig. 16 is a fragmentary perspective view of the completed article as applied to an automobile front frame.

Referring in detail to the drawings, 1 in Fig. 1 represents a suitable first operation male die and 2 a cooperating female die. The male die may consist of an enlarged upper end portion 3 providing a shoulder 4, the reduced lower end 5 of this die conforming substantially to the inside diameter of the tube indicated at T. The female die, as shown, has an upper enlarged recess 7 connected by tapering surfaces 8 with a reduced recess 9 substantially fitting the exterior of the tube and laterally supporting it. The particular male die herein shown is provided with irregular shoulder portions 100

consisting of a pair of projections 10 for forming flange stock for flanges such as shown in Fig. 10. Incidentally, if a flange such as shown in Fig. 14 is desired no such enlargements 10 would be used.

5 It will be noted in Fig. 1 that the reduced portion 5 of the male die extends slightly beyond the tapering surface 8 of the female die before the projections 10 come into contact with the upper end of the tube. One 10 result of thus supporting the tube interiorly and exteriorly, at a point below the tapered surface, is that when the compression starts, the upset metal of the tube is wedged between such tapering surface and the male die, thus 15 effectually preventing downward movement of the tube and preventing the tube from buckling inwardly under the severe compression blow given the upper end of the tube. The action of upsetting the end of the tube 20 is of course quite rapid in order that the flow of metal will be uniform and in order to preserve all of the heat. Nevertheless the projections 10 do not have a tendency to split 25 the end of the tube, but merely shove the metal of the tube downwardly beneath them, changing the character of the metal from 30 that of a straight grained tube into a compressed grained tube, the grains lying in irregular undulations and greatly compressed 35 together, as in all other parts of the upset portion. Incidentally the metal of the upset portion is strongest at the bottoms of such depressions by reason of being more highly compressed, this being very desirable in order to overcome any tendency of the finished 40 bracket to split apart between the flanges.

Fig. 4 shows the end of an upset tube when 45 made by the dies formed as just described, the upset portion being indicated at  $t$  and the tapered reinforce at  $T_1$ . The reason for 50 this particular shape is that when the flanges are made for the front portion of an automobile frame it is desirable to have one narrow flange for receiving a single bolt and a wider flange for receiving more than one. Any 55 number or shape of flanges may be so started by the male upsetting die. For example, as shown in Fig. 5, the depressions  $t_2$  are substantially 60 diametrically opposite, wherefore the flange stock portions  $t_1$  between the depressions are practically alike; this blank being used in forming such a bracket as shown in Figs. 13 and 14. If it is desired to 65 form a single annular bracket, such as shown in Fig. 15, the blank may be made substantially as shown in Fig. 6.

For the second and final operation, we 70 may place the blank in a female die; such 75 for example as indicated at 20 in Fig. 8, preferably with the upper edge of the tapering portion  $T_1$ , substantially even with a depressed surface 21 of this die. In order to 80 more precisely determine the shape of the flanges the sides 22 of the female die con-

tiguous with the surface 21, may conform substantially to the desired flange shape. Fig. 7 shows a suitable male finishing die which may comprise a body portion 25, conforming substantially to the flange shape of 70 determining recess in the female die, and which may have a projection 26 adapted to interiorly support the upset tube during the flanging operation. As shown in Fig. 8 the male die has started to compress and flow the 75 flange stock portions  $t_1$  between the depressions  $t_2$ .

If desired, we may form additional reinforce members such as webs  $T_4$ , Fig. 13, these webs being forced outwardly from the upset metal into recesses such as shown at 28 in the female die block 20a in Fig. 11. Any number, shape or size of such flanges may be formed as required. Fig. 11 shows a web  $T_4$  being formed into a recess 28, the grain of the metal in such case being found to bridge 85 from the tapered reinforce portion  $T_1$  to the flange, thus securing additional strength.

In Fig. 14 we show an additional refinement consisting of machine pads  $T_5$  connected by a ridge  $T_6$  extending along the periphery of the flanged bracket. These pads and ridges may be formed by providing corresponding depressions at the bottom of the recess such as 27 in the male finishing die.

Referring again to Figs. 6 and 15 which show respectively blank and finished articles formed thereby, it will be noted that the walls of the upset portion are made heavy as by upsetting a longer portion of tube. This is desirable since such an annular flange will take more material than the forms shown in either Figs. 12 or 13. If desired this annular flange may also be provided with any 100 number of bracing webs  $T_4$ .

One form of finished article is shown in Fig. 16 wherein  $F$  represents the forward portions of an automobile frame, these portions being held rigidly together by the tube 110  $T$  and flanges  $T_2$  forged thereon, the flanges being bolted to the web portions of the frame in the usual manner.

From the above description it will be seen 115 that we have provided a process for forming articles, such as automobile cross frame braces, which may be all one piece and in which the metal in the flanges, the connecting reinforcing taper and the webs is of substantially 120 different character than that of the tube, the latter consisting of drawn or possibly seam welded tubing with the grain running substantially parallel, while the bracket portion which consists of forged material 125 is therefor more rigid and stronger than if made by merely turning out flanges of the same side wall. While we have described in detail the characteristics of the various dies, it is to be understood that we may utilize dies made up of any number of sections 130

and in any suitable form which we may find practicable, and we do not wish to be otherwise limited to unessential details.

We claim:

- 5 1. The process of forming a hollow flanged unit from tubing comprising heating the end of a section of such tubing, supporting the tubing, upsetting the heated end to thicken and compress it, simultaneously de-
- 10 pressing a portion of the heated stock in an axial direction beyond the adjacent portions to form flange stock, and thereafter forming laterally extending flanges from such stock.
- 15 2. The process of forming a flanged tube, comprising, heating the end of a suitable section of metal tube stock, supporting and forcibly compressing the end of the heated tube to thicken it, separating the thickened end into flange stock by endwise compression
- 20 at certain portions of the end of the tube to a greater extent lengthwise of the tube than at other portions, and then spreading the flange stock into predetermined spaces by further endwise compression on said flange
- 25 stock, to finish form the flanges.

In testimony whereof, we hereunto affix our signatures.

CLINTON W. STOVER.  
HARRY WOODHEAD.

30

35

40

45

50

55

60

65